

Apr. 17, 1923.

1,452,120

R. LAMB

COMPENSATING FILLER FOR BLOCK PAVING

Filed March 11, 1920

Fig. 1.



Fig. 2.



INVENTOR

Richard Lamb

## UNITED STATES PATENT OFFICE.

RICHARD LAMB, OF NEW YORK, N. Y.; SARAH E. LAMB, EXECUTRIX OF SAID RICHARD LAMB, DECEASED, ASSIGNOR TO SARAH E. LAMB.

## COMPENSATING FILLER FOR BLOCK PAVING.

Application filed March 11, 1920. Serial No. 365,091.

*To all whom it may concern:*

Be it known that I, RICHARD LAMB, a citizen of the United States, and a resident of New York, in the county of New York and State of New York, have invented an Improvement in Compensating Fillers for Block Paving, of which the following description is a specification.

This invention relates to a novel composition of matter and process for making it and its combination with wood blocks forming a floor or paving for road beds having novel structural and functional characteristics. The novel combination of the constituent elements of the composition herein-after referred to give to it characteristics which especially adapt it for use as a filling material between adjacent wood blocks of a floor or pavement. It may be easily applied in plastic or fluid condition but when dry becomes hard and adheres to the blocks and holds them in proper position but in case water comes in contact with the floor or pavement and the blocks become wet and expand, the composition filler also absorbs the water and thereby becomes soft and yielding and the expansion of the blocks is thus permitted without buckling of the floor or pavement, as would otherwise occur. When the blocks gradually dry the filler does also and becomes hard again. It, therefore, constitutes what may be called a compensating filler or compound. In applying the liner, any surplus on the face of the blocks may be easily and completely removed. The composition has the advantage over the use of sand as a filler in that the sand is not adherent and works its way down under the blocks, not only making the surface uneven but ceasing to serve properly as a filler, whereas the present composition is adherent and is always in place and yields when required under the expansion due to moisture. It has the advantage over the use of pitch or asphalt as a filler in that they get soft in hot weather and are pressed out on the upper surface of the blocks and because of their sticky nature that is very objectionable, aside from the fact that the filler does not remain in proper position to act as a filler. The present composition does not soften by hot weather and even if some of it

by chance gets on the surface of the floor or pavement, it is not objectionable and may be removed easily or will wear off naturally, 55 since it will not stick to things coming in contact with it. Pitch and asphalt do not soften, when wet, to permit expansion of the blocks and it is impossible to thoroughly remove any which works out on 60 to the surface. The present composition has the advantage over the use of sand and cement grout, not only because that requires several days delay for forming before using, while the present composition dries in about 65 twenty-four hours but because the sand and cement grout do not become soft, when wet, and thus either do not yield to permit expansion or are disintegrated. If the blocks shrink after the grout is set and hardens, 70 it never becomes soft so as to settle or flow outwardly filling the space between blocks, as does the present composition but there is a looseness between blocks. The novel features of the invention will be more fully 75 understood from the following description and claims taken with the drawings.

In the drawings—

Figure 1 is a perspective view partly broken away of a floor construction embodying the invention, and

Figure 2 is a similar view showing a modified form of leveling base on which the wooden blocks rest.

The composition constituting one of the 85 main features of this invention embodies ar-gillaceous sand, clay and a colloidal agent, preferably lignosulfonate.

Lignosulfonate is a bi-product of the sul-fite or bisulfate process for making wood 90 pulp. In digesting the wood about one half of the wood remains in the digestor as "cel-lulose," which is paper pulp. The remainder is a solution known as sulfite or waste liquor, and is called technically lignosulfonate. It 95 is not of bituminous or oily nature, and is practically odorless and is clean. It can therefore be used on floors where pitch or asphalt would be objectionable.

It is generally believed by scientific road builders that the wetting of road materials form colloids that produce a strong bond. The lignosulfonate is rich in colloidal ex-tractive matter, and when used simply has-

tens nature's method of bonding road material. Lignosulfonate is commonly used for this purpose in road construction. The object of its use heretofore has been to make 5 as far as possible permanently solid the material of the road bed, it not being desired ever to have the bond soften and harden again as in my invention.

The argillaceous sand used in making the 10 composition may be formed from iron blast furnace slag, lime stone, gneiss, feldspar or other siliceous stones and the clay is preferably a kaolinite, in other words, hydrous aluminum silicate, and the clay should constitute about fifteen per cent by volume of 15 the mixture of sand and clay. Pulverized solid lignosulfonate is intimately and thoroughly mixed with the mixture of sand and clay in approximately the proportion by 20 volume of one to twenty-five, so that the resulting mixture contains about four per cent of lignosulfonate. This mixture, when wet, becomes a soft and plastic mass which, after 25 drying, is solid and hard but even after drying and hardening it will again absorb water if brought in contact with it and again become soft and plastic. In some localities 30 argillaceous sand of the proper kind containing the desired proportion or percentage of clay may be found in nature and it may of course be used without the admixture of additional clay from outside sources. The 35 complete mixture as a dry composition, including all of the ingredients above stated, may be made and sold to those wishing to use it for lining paving blocks or for analogous purposes. Since, however, siliceous sand, suitable for mixing with the clay and lignosulfonate, may be found in most localities, it is preferable for some reasons and 40 under some conditions to omit the sand in forming the mixture, using only clay or kaolin and about thirteen and one-half per cent by volume of lignosulfonate, intimately 45 mixed. The purchaser and user of the composition may then add the content of sand indicated above and thoroughly mix the material before using.

In practically applying the composition as 50 a compensating filler for the wood blocks of a pavement in the embodiment shown in Figure 1, a concrete base 5 is first formed on which is laid a cushion 2 of dry cement and sand pressed into the form of a layer with 55 a smooth flat upper surface. The cushion is then sprinkled with water and the wood blocks 3 are placed in position on it close together. Since wood blocks such as shown usually shrink laterally and longitudinally 60 after being cut to form, according to the moisture in them, they should be permitted to dry and shrink to the desired extent before taking the step of applying the composition as a filler. After the blocks are in 65 proper position and condition, the mixture

above described may be forced into the spaces between blocks as a compensating filler in two ways. The dry mixture may be made to enter and fill the spaces indicated at 1 and water is then poured on the filler material between the blocks until it is saturated with water and becomes a plastic mass. It is then allowed to stand undisturbed and to dry and after drying it is hard and solid and properly holds the blocks in place. Instead of filling the spaces between blocks with dry mixture and later adding water, the mixture may be first mixed with water until it has a consistency which will permit it to flow readily down between the blocks, filling the spaces under slight squeezing pressure applied to it.

Another method for applying the filler is to form it in situ between the wooden blocks. In this case a mixture of dry sand and clay in proper proportions is inserted between the blocks and liquid lignosulfonate with about one and one half times its volume of water is poured into it between the blocks and being very fluid, it will penetrate all parts of the sand and be thoroughly and uniformly distributed throughout the filler. The filler, when in place, will set and become hard at any temperature but at a temperature below 60 Fhr., if not again wet will dry and harden in twenty-four hours. After it has become hard, it will remain so unless water is applied to it but if water is applied, it will again become plastic. It follows, therefore, that if the blocks shrink after it has become hard, an application of water to it will make it soft so that it will flow and fill the space between blocks. If after hardening the blocks have water applied to them and expand, the 95 filler receiving the water becomes plastic and yields. My compensating filler is not affected by machine oils or gasoline which are often found upon streets and factory floors and, as heretofore stated, contains no oily or sticky material which is objectionable and cannot be easily removed from the floor surface when it happens to be on that surface.

The embodiment or use of the invention disclosed in Figure 2 differs from that indicated above only in the composition of the cushion marked 4 which takes the place of that marked 2 in Figure 1. The cushion 4 is formed of low melting point pitch pressed into position on the concrete base 5.

This pitch should be preferably of from 130 to 140 deg. Fhr. and should be allowed to cool before placing the blocks upon same.

The blocks should be laid close together upon the cold pitch which will hold the blocks tightly to the concrete bed. After the blocks have shrunk the compensating filler should be applied as before described. If the floor is subject to constant wetting, 125 paraffine oil or other material that will make 130

the surface non-hygroscopic can be used on the surface to shed the water.

Having thus described the invention what is claimed as new and desired to secure by 5 patent is:

1. The combination with paving blocks, of a support therefor, and a filler between adjacent blocks composed of an intimate mixture of colloidal agents, argillaceous sand and 10 clay in such proportions that the filler will be solid and hard when dry and soft and yielding when wet.

2. The combination with paving blocks, of a support therefor, and a filler between adjacent blocks composed of an intimate mixture of lignosulfonate, argillaceous sand and 15 clay in such proportions that the filler will be solid and hard when dry and soft and yielding when wet.

20 3. The combination with paving blocks, of a support therefor, and a filler between adjacent blocks composed of an intimate mixture of lignosulfonate, argillaceous sand and 25 clay, the lignosulfonate constituting approximately four per cent of the mixture by volume.

4. The combination with paving blocks, of a support therefor, and a filler between adjacent blocks composed of an intimate mixture of lignosulfonate, argillaceous sand and 30 clay, the lignosulfonate constituting approximately four per cent of the mixture by volume, and the clay constituting approximately fifteen per cent of the remainder by volume.

35 5. A composition of matter comprising an

intimate uniform mixture of fine grained argillaceous sand and approximately fifteen per cent by volume of clay and approximately four per cent by volume of pulverized solid lignosulfonate.

6. A composition of matter adapted for use in forming a filler for paving blocks comprising an intimate mixture of kaolin clay and approximately thirteen and one half per cent by volume of pulverized solid ligno- 40 sulfonate. 45

7. The process of making and applying a filler for paving blocks, comprising thoroughly mixing fine grained argillaceous sand containing clay and lignosulfonate in such 50 proportions that when wet the mixture will be soft and plastic and when dry hard and solid pouring said mixture between the blocks to fill the spaces with sufficient water to make it plastic and allowing it to dry. 55

8. The process of making and applying a filler for paving blocks, comprising interposing in the spaces between adjacent blocks a composition comprising argillaceous sand and approximately fifteen per cent by volume 60 of clay and approximately four per cent by volume of lignosulfonate, the said substances being thoroughly and uniformly distributed throughout the mixture together with sufficient water to render the mixture plastic. 65

In testimony whereof I affix my signature, in the presence of a witness.

RICHARD LAMB. [L.S.]

Witness:

LAURA E. SMITH.